

Jan. 5, 1965

J. L. DEWEY

3,163,895

CONTINUOUS CASTING

Filed Dec. 16, 1960

4 Sheets-Sheet 1

FIG. 1



INVENTOR.  
JOHN L. DEWEY

BY  
*Robertson & Smythe*  
ATTORNEYS

Jan. 5, 1965

J. L. DEWEY

**3,163,895**

## CONTINUOUS CASTING

Filed Dec. 16, 1960

4 Sheets-Sheet 2

FIG. 2



INVENTOR.  
JOHN L. DEWEY

BY  
Robertson & Smythe  
ATTORNEYS

Jan. 5, 1965

J. L. DEWEY

3,163,895

CONTINUOUS CASTING

Filed Dec. 16, 1960

4 Sheets-Sheet 3

FIG. 4



FIG. 3

INVENTOR.  
JOHN L. DEWEY

BY  
*Robertson & Smythe*  
ATTORNEYS

Jan. 5, 1965

J. L. DEWEY

3,163,895

CONTINUOUS CASTING

Filed Dec. 16, 1960

4 Sheets-Sheet 4



INVENTOR.  
JOHN L. DEWEY

BY  
*Robertson & Smythe*  
ATTORNEYS

1

3,163,895

## CONTINUOUS CASTING

John L. Dewey, Florence, Ala., assignor to Reynolds Metals Company, Richmond, Va., a corporation of Delaware

Filed Dec. 16, 1960, Ser. No. 76,236  
7 Claims. (Cl. 22—57.2)

This invention relates to the continuous casting of aluminum ingot of a purity exceeding that of the molten feed metal.

For a long time there has existed the need for commercial aluminum ingot of high purity to satisfy the demand for high purity aluminum to be used in electric conductors and condensers, petroleum catalyst supports, corrosion-resistant chemical equipment, hardware, automotive trim, and, more recently, for use in nuclear reactor installations. The only process capable of supplying these needs heretofore has been the well known three-layer refining cell process and its modifications. This process, comprising the electrolytic refining of a copper-aluminum alloy in a fused salt bath at 730-780° C., is presently in use throughout the world in spite of the fact that it costs nearly as much to refine a pound of metal as it does to produce the pound of metal initially from unmined bauxite. While many attempts have been made over the years to find a low-cost process to replace the expensive refining cell process, three-layer electrolytic refining has remained the one answer to today's commercial needs notwithstanding its inherently high cost burden. Substitute processes have proved useful only for laboratory purposes or in small-scale production of the high purity metal, and they too have imposed a high cost of production either because they require elaborate apparatus and a multiplicity of operating steps, or are not well adapted to continuous production methods, or are not capable of producing uniform high purity throughout the length of a continuously cast ingot, or for other reasons known to those who have been concerned with the problem. So, while some of these processes have found use in the purification of semi-conductor materials which sell at hundreds of dollars a pound, they are not continuous, seldom produce a uniform product, and are neither physically nor economically suitable for the purification of large quantities of low-cost metals, such as aluminum.

## SUMMARY

I have discovered a way to produce by a continuous casting method and apparatus, aluminum ingot having throughout its length a purity continuously maintained at a substantially uniform level above the purity of the molten feed metal. The production of this high purity, homogeneous ingot in commercial sizes according to my discovery can be accomplished at only a fraction of the cost of electrolytic refining. I have also found that these ingots can be produced in any desired degree of purity by changing the production rate or the feed stock, so that the cost of production is in direct relation to the desired purity.

According to my invention molten metal is fed into the inlet of a pass-through mold in which a portion of the metal is frozen and the frozen portion is continuously withdrawn from the outlet of the mold. At the same time, the molten portion of the feed metal is caused to flow rapidly over the interface between the molten and frozen metal, as by stirring, and concurrently there is withdrawn from the mold as casting progresses molten metal including metal which has flowed over the interface and contains a higher percentage of impurities than is present in the feed metal. The relationship between (a) the rate of feeding the molten metal, (b) the rate of withdraw-

2

ing the solid portion from the mold and (c) the rate of withdrawing molten metal from the mold, is adjusted so that each rate is maintained substantially constant relative to the others. This serves to maintain a substantially uniform composition of the molten metal just above the interface with a resultant uniformity in purity of the ingot produced. However, the rates can be increased or decreased as desired with purity of product changing inversely with the rate of production. As an example, I have produced 8-inch diameter ingots, a size and shape commonly used for extrusion billets, from feed stocks of different purities at various production rates as shown in Table 1:

Table 1

| Run No. | Production Rate, lbs./hr. | Composition, Percent Aluminum |         |
|---------|---------------------------|-------------------------------|---------|
|         |                           | Feed                          | Product |
| 20      | 5                         | 99.90                         | 99.983  |
|         | 45                        | 99.90                         | 99.97   |
|         | 7½                        | 99.87                         | 99.976  |
|         | 10                        | 99.87                         | 99.966  |
|         | 15                        | 99.87                         | 99.961  |
|         | 17½                       | 99.87                         | 99.956  |
| 25      | 5                         | 99.78                         | 99.93   |
|         | 7                         | 96.1                          | 98.4    |

Production equivalent to Run No. 7, if performed by the three-layer electrolytic refining process would require a specially constructed fused salt electrolytic cell, 62,000 amperes D.C. electricity with attendant rectification and distribution equipment, in addition to a direct chill casting unit to produce the ingot.

## DESCRIPTION

With reference to the accompanying drawings I shall now describe the best mode contemplated by me for carrying out my invention.

FIG. 1 is a view showing the casting and purification apparatus of FIG. 2 to an enlarged scale.

FIG. 2 is an elevational view, partly in section, showing the general arrangement of a plant embodying apparatus constructed and operated according to my invention.

FIG. 3 is an exploded perspective view of the stirrer for the casting unit.

FIG. 4 is a diagram showing percentage removal of metallic impurities in a typical run.

FIG. 5 is a diagram showing total impurity distribution lengthwise of the ingot product.

FIG. 6 is a diagram showing total impurity distribution transversely of the ingot product.

The continuous direct chill ingot casting apparatus constructed according to my invention and used in practicing my improved method comprises in its general arrangement the following principal parts: a pass-through molding chamber 10 having an inlet and an outlet spaced longitudinally thereof, means which may include a heated pipe 11 for feeding molten metal into the upper end, or inlet, of the molding chamber, means which may include a water spray 12 for freezing a portion of the feed metal, means which may include an ingot lowering device 13 for continuously withdrawing the frozen portion from the lower end, or outlet, of the molding chamber, means which may include a stirring device 14 for causing the molten portion of the feed metal to flow rapidly over the interface between the molten and frozen metal, and means which may include a heated overflow pipe 15 for continuously withdrawing from the molding chamber molten metal including metal which has flowed over the interface and contains a higher percentage of impurities than is present in the feed metal. Stirring as by means of the stirring de-

vice 14 is performed in a manner that causes the molten metal adjacent the interface to rotate around the axis of the ingot while being drawn downwardly against the peripheral portions of the interface, thence inwardly toward said axis and upwardly away from central portions of the interface in the general manner indicated by the arrows in FIG. 1.

Proceeding to a more detailed description of my invention as exemplified by its practice during a typical pilot plant operation performed under my direction, I now disclose several specific examples utilizing a preferred form of my continuous casting apparatus with its improved means for maintaining a uniform rate of purification with resultant uniformity in purity of ingot produced.

EXAMPLE 1

Fifty-pound pigs 16 of aluminum feed metal approximately 5" x 6" x 28" long were tied onto an endless chain 17 by means of  $\frac{3}{8}$ "-diameter high purity aluminum rod 18. The chain was suspended over the melt crucible 19 by a sprocket 20 which in turn was connected through a gear system 21 to a variable speed motor (not shown) in such manner that the rate of rotation of the sprocket, and hence the rate of movement of the chain, could be accurately controlled. As the sprocket revolved, the pigs 16 attached to the chain were lowered at a constant rate into the pool of molten aluminum 22 in the crucible, causing the level of the molten aluminum to rise above the inlet 23 of overflow pipe 11 so that liquid aluminum flowed through the overflow pipe to the mold 10 of the casting unit. As the pigs 16 contacted molten metal in the crucible, they melted progressively from the lower end and were in due time completely released from the chain by melting of the  $\frac{3}{8}$ " aluminum rod. When the pigs had been partially lowered into the melt additional pigs were hung from the chain in the same manner and spaced so as to maintain the total volume of aluminum at each point along the chain reasonably constant. Thus the rate of displacement of the molten aluminum into the overflow pipe 11 was substantially constant.

The melt crucible 19 was a standard clay graphite tilting furnace crucible. It sat within a gas-fired furnace consisting of a silicon carbide tile combustion chamber 25, an outer steel shell 26 and a layer of thermal insulation 27 disposed therebetween. The firebrick bottom 28 of the furnace was covered with a layer of silicon carbide cement and the top cover 29 of the furnace was cast from "Purotab" alumina casting mix (approximately 85% tabular alumina, 15% high-purity calcium aluminate).

A control thermocouple 30 was placed between the silicon carbide tile and the insulation in the position shown. The signal from this thermocouple was read out on a standard potentiometer-type recorder which also supplied a signal to a standard type of proportioning controller (not shown) which actuated a conventional servo motor arranged to operate the control valve of a gas burner 31 in accordance with the deviation of the furnace temperature from its set point.

The overflow pipe 11 was constructed from a clay graphite tube spaced within a tube 32 of silicon nitride bonded silicon carbide covered exteriorly with suitable thermal insulation. Hot combustion gases from the cast furnace 33 exhausted through the annular space 34 between the two tubes, maintaining the temperature of the clay graphite tube 11 above the melting point of the feed metal. The clay graphite tube and the clay graphite crucible 19 were shaped to form a ball and socket joint 35 which was covered with a thick layer of alumina casting mix to prevent the joint from leaking. The opposite end of the tube was suspended over the upper portion of the cast unit so that aluminum feed flowing from the melt furnace through the overflow pipe flowed into the open top 36 of the mold 10.

The cast unit mold 10 was constructed in the form of a vertically disposed graphite tube of 8" inside diameter mounted within a tubular clay graphite member 37 situ-

ated within the gas-heated cast furnace 33 of a construction similar to that of the melt furnace 24. A stirrer assembly 14 was suspended within mold 10. The interior lip of the bell shaped upper end of mold 10 was filled with alumina casting mix 38 to provide protection from air burning above the molten aluminum level. The clay graphite overflow pipe 15 was attached to the graphite mold tube by a ball and socket joint 39 sealed in alumina casting mix. Molten aluminum overflowed through the pipe 15 into a crucible 40 exteriorly of the furnace for removal from the plant as an overflow product. The clay graphite member 37 had a lower end 41 of reduced size which extended downwardly through an opening 42 in the steel floor 43. The upper part of clay graphite member 37 was bonded to the graphite mold tube 10 with a commercial graphite cement to provide a good flow of heat from the clay graphite into the graphite; the lower end 41 of member 37 was spaced slightly from mold 10 and this space was filled with a commercial thermal insulation material comprising ceramic fibers with an inorganic binder known as "Fiber-Frax" cement. The furnace 33 was fired by a gas burner 44. A Chromel-Alumel control thermocouple 74 was maintained in a hole in the clay graphite member 37 in the position shown in FIGS. 1 and 2 to give a sensitive control of the temperature of the casting furnace. The signal from this thermocouple was read out on a potentiometer-type adjustable zero adjustable range recorder adjusted for a full-scale range of 2 mvs. The recorder supplied a signal to a proportioning type controller which actuated a servo motor that positioned a gas control valve in accordance with the deviation of the control point temperature from its set point. The temperature variation during normal operation was  $\pm\frac{1}{4}$  °C. at the thermocouple junction.

The stirrer assembly 14 consisted of a C.S. grade graphite impeller section 45, a clay graphite shaft 46, drive means 47 for turning the shaft and impeller at predetermined constant speeds and means 48 for adjusting the vertical position of the stirrer assembly. The graphite impeller (FIG. 3) was cut from a 7" diameter x 12" long C.S. grade graphite piece to provide a solid 4" diameter center shaft 49 with four impeller blades 50 at its lower end. Each blade extended 4" along the shaft, was inclined 45° from the vertical, was about 1" thick, and extended outward from the hub 1 $\frac{1}{4}$ " at 0°, 90°, 180° and 270°. A 6 $\frac{1}{2}$ " I.D. x 7" O.D. x 4" high graphite sleeve 51 was fitted around the extremities of the blades and held in position with graphite plugs flush with the outside surface of the sleeve. The upper end of shaft 49 was provided with a screw thread connection to the clay graphite shaft 46 secured to a steel collar 52. The collar in turn was welded to a steel shaft 53, containing an elongated keyway 54. The shaft 53 extended through bearings 55 and was suspended by a cable 56 extending through a pulley 57 directly along the center line of the mold 10. Shaft 53 was keyed to the drive pulley 58 in a manner to permit the shaft to move vertically with respect to the pulley. The pulley was connected through a V-belt to a variable speed motor 59 having infinitely variable speed settings between 55 and 550 r.p.m.

The product ingot 60 was lowered from the casting unit through the bottom end of the mold 10 by means of the hydraulic lowering device 13. The ingot shrank on cooling from the 8" diameter of the mold at the interface to about 7 $\frac{1}{16}$ " diameter at its cool end. The freezing interface was usually about 16" up from the bottom of the mold. The water spray ring 12, positioned 10" below the bottom of the mold, consisted of a 1 $\frac{1}{2}$ " pipe bent to form a 12" I.D. circle with sixty-four  $\frac{1}{16}$ " diameter holes equally spaced along the intersection of a horizontal plane through the circle such that the water jets were inclined downward about 30° from the horizontal plane. Water rate to the spray ring was metered.

The hydraulic lowering device 13 consisted of two sets of three-point clamps, each set built into horizontally

disposed steel platforms 61, 62, supporting hydraulic cylinders 63, 64, for opening and closing the clamps and supported by vertically disposed hydraulic cylinders, 65, 66, respectively, for which the rate of downward movement was controlled and kept constant by withdrawing fluid from the supporting cylinders at a constant rate with a metering pump. Pushbutton-type hydraulic valves 67, 68, placed so as to be operated according to the respective positions of the platforms when near the extremities of the platform motion controlled the fluid flow directions from an auxiliary hydraulic pump and accumulator system (not shown) so that at least one of the sets of clamps was engaging the ingot and lowering at all times. When the upper platform neared the end of its downward travel it contacted a pushbutton which started a sequence of operations, viz:

- (1) The clamp set on the lower platform closed to engage the ingot.
- (2) The lower platform started downward movement at the same rate as the upper platform.
- (3) The clamp set on the upper platform opened to free the ingot.
- (4) The upper platform raised to its initial level.
- (5) The upper platform contacted a second control button.
- (6) The clamp set in the top platform closed to engage the ingot.
- (7) The top platform began a downward motion at the same rate as the lower platform.
- (8) The clamp set on the lower platform opened.
- (9) The lower platform rose to its original position.

The ingot was therefore lowered continuously at a constant controlled rate, which rate could be changed by changing the stroke length of the metering pump. This type of lowering mechanism is described and claimed in the copending application of Robert F. Treadway and Billy K. Davis, Serial No. 120,540, filed June 29, 1961.

The cutoff band-saw 69 consisted of a pair of wheels 72 mounted on axles 73 disposed parallel to each other and inclined upward 4° to the horizontal, one axle lying free in its bearings and the other axle engaging a motor driving the band-saw blade at forty feet per second. The whole was suspended on a platform mounted on a fixed track and wheels so that the saw blade, which was held in place on the wheels by a pair of band-saw guides, could be pushed through the ingot to complete a cut as at C. The band-saw blade was a 1/2"-wide skip-tooth blade having four teeth per inch. A maximum length of 17" could be cut from the ingot on one saw cut. Cuts were made without stopping the ingot lowering.

To start casting, a 7 3/4" diameter ingot was pulled into mold 10 by means of an eye bolt in the top of the ingot and was clamped into the lowering device 13, so that the top of the ingot was about even with the overflow pipe 15. The cast unit gas burner 44 was ignited and the controller set to maintain a temperature of 871.0° C. at the junction of thermocouple 74. Four hundred pounds of 99.90% aluminum was placed in the melt furnace 24, the gas burner 31 ignited and the controller set to hold the melt furnace temperature at 775° C. The setting of the variable drive motor on the pig lowering unit was adjusted to give a lowering rate of the feed pig 16 of 11.2" per hour. The stroke length of the metering pump of the lowering device had been previously adjusted to give a lowering rate of the ingot 60 of 1.0 inch per hour. After about eight hours, when the melt furnace crucible 19 was full of molten aluminum and the ingot 60 had melted down a distance of about 10" below the overflow pipe 15, the cooling water was turned on at a rate of about 11.8 cu. ft. per hour, the stirrer 14 was lowered into the molten aluminum with the bottom of its impeller 45 about 3" above the liquid-solid interface 70 and started rotating at 200 r.p.m. The bulk liquid temperature in the cast unit at this time was about 665° C.

Lowering of the feed pigs 16 was then started. As soon as molten aluminum began overflowing through the overflow pipe 15 into the overflow crucible 40, the lowering device 13 was started. Throughout the above period the level of the liquid-solid interface 70 with respect to the mold 10 was measured every fifteen minutes by probing between the stirrer blades with a 1/2" diameter graphite rod with the stirrer momentarily shut off. About a half hour after the start of ingot lowering, the stirrer assembly was lowered again so that the bottom of the stirrer was approximately 1" above the liquid-solid interface. The position of the interface was then checked every hour with the graphite probe rod and the stirrer was raised or lowered when necessary to keep it 1" above the interface. It was found that the stirrer was sufficiently free to ride up with the interface during an upset so that although there were occasions when the stirrer actually rubbed on the interface it did not break or become embedded in the frozen aluminum. Normally the interface was quite stable at about the level of the furnace floor. Feed pigs 16 were tied to the feed chain as needed to maintain by displacement a flow rate through the casting unit of 40 lbs./hr. Overflow crucibles 40 were changed as needed to provide a receptacle for the overflow product amounting to 35 lbs./hr. When the ingot 60 had been lowered 10 to 15" below the cutting line of the cutoff saw 69, the section 71 of the ingot was cut off by manually pushing the saw assembly so that the band-saw blade cut its way completely through the ingot.

After twenty-four hours of operating under the above described conditions, the temperature of the aluminum overflowing from the melt furnace was 728° C., and the bulk liquid temperature in the cast unit was 672° C. Inlet water to the spray ring 12 was 15° C. and the runoff from the ingot was about 30° C.

When it was desired to shut the plant down, lowering of the feed pigs 16 was stopped, the lowering device 13 was shut off, the stirrer 14 was removed from the cast unit, cooling water was stopped and finally the gas burners 31 and 44 were shut off. Molten aluminum in the mold 10 was allowed to freeze in place to form a portion of the starting ingot for a subsequent run. Similarly, molten aluminum in the melt furnace 24 was allowed to freeze in place.

Eighty-three inches of high-quality ingot were made during the particular pilot run here described. Analyses showed that the impurity levels in the product were substantially less than in the feed, for instance, silicon 87% less, iron 94% less, copper 84% less, magnesium 67% less, zinc 45% less, and gallium 55% less. See FIG. 4. Average analyses of the Product, Feed, and Overflow were:

| Impurity Element | Feed, p.p.m. | Product, p.p.m. | Overflow, p.p.m. |
|------------------|--------------|-----------------|------------------|
| Silicon.....     | 348          | 46              | 395              |
| Iron.....        | 420          | 25              | 469              |
| Copper.....      | 18           | 3               | 19               |
| Magnesium.....   | 9            | 3               | 7                |
| Zinc.....        | 68           | 37              | 71               |
| Gallium.....     | 71           | 32              | 86               |

The distribution of the total impurities in the product ingot lengthwise of the eighty-three inch section is shown in FIG. 5. In this view each point shown by the graph represents the average of spectrographic analyses at between ten and seventeen points located in the same transverse plane. FIG. 6 shows distribution of total impurities transversely of the ingot. In this view each point shown by the graph represents the average of spectrographic analyses at about twenty-two points located at the same distance from the ingot center. The shaded areas in FIGS. 5 and 6 extending two standard deviations [2σ] on each side of the average represent the ranges within which statistical analysis of the data indicates that about 95% of all impurity analyses will fall.

7  
EXAMPLE 2

In the manner described in Example 1, 19.7 lbs. per hour of 96% Al feed was passed through the cast unit and split into 7.0 lbs. per hour of approximately 7 $\frac{3}{4}$  inch diameter ingot and 12.7 lbs. per hour of overflow product. The ingot lowering rate was 1.4 inches per hour, the stirrer rate was 204 r.p.m., the distance between the liquid-solid interface and the bottom of the stirrer averaged 6.8 inches, and the cast unit control temperature was 878° C. The following average analyses were obtained over 55 inches of a continuous section of ingot:

| Impurity Elements | Feed, p.p.m. | Product, p.p.m. | Overflow, p.p.m. |
|-------------------|--------------|-----------------|------------------|
| Silicon.....      | 16,500       | 7,400           | 21,800           |
| Iron.....         | 16,200       | 5,500           | 19,900           |
| Copper.....       | 5,700        | 2,400           | 6,900            |
| Zinc.....         | 230          | 200             | 360              |

## EXAMPLE 3

In the manner described in Example 1, 33.3 lbs. per hour of 99.78% Al feed was passed through the cast unit and split into 5.4 lbs. per hour of approximately 7 $\frac{3}{4}$  inch diameter ingot and 27.9 lbs. per hour of overflow product. The ingot lowering rate was 1.1 inches per hour, the stirrer rate was 200 r.p.m. and the distance between the liquid-solid interface and the bottom of the stirrer averaged 2.9 inches. The following average analyses were obtained over 92 inches of a continuous section of ingot:

| Impurity Elements | Feed, p.p.m. | Product, p.p.m. | Overflow, p.p.m. |
|-------------------|--------------|-----------------|------------------|
| Silicon.....      | 917          | 199             | 967              |
| Iron.....         | 934          | 112             | 1,035            |
| Copper.....       | 19           | 8               | 28               |
| Magnesium.....    | 3            | 3               | 2                |
| Zinc.....         | 257          | 169             | 235              |
| Gallium.....      | 38           | 60              | 43               |

## EXAMPLE 4

Additional gas burners were added to the melt furnace to provide a melting rate of 250 lbs. per hour. Feed of 99.9% Al was then passed through the cast unit at a rate of 250 lbs. per hour, where it was split into about 45 lbs. per hour of approximately 7 $\frac{3}{4}$  inch diameter ingot and about 205 lbs. per hour of overflow product. The ingot lowering rate varied between 8 and 10 inches per hour, the distance from the liquid-solid interface to the bottom of the stirrer was about 8.5 inches, the cast unit control temperature was 778° C., temperature of the molten feed to the cast unit was about 670° C., the solid-liquid interface was 24 inches below the overflow pipe 15, and the stirrer rate was 200 r.p.m. Average analyses over 30 inches of ingot were as follows:

|         | Feed, p.p.m. | Product, p.p.m. | Overflow Product, p.p.m. |
|---------|--------------|-----------------|--------------------------|
| Fe..... | 350          | 116             | 390                      |
| Si..... | 400          | 91              | 410                      |
| Cu..... | 15           | 10              | 18                       |
| Zn..... | 120          | 40              | 140                      |
| Ga..... | 90           | 33              | 100                      |

## EXAMPLE 5

In the manner described in Example 1, 16.7 lbs. per hour of 99.87% Al feed was passed through the cast unit and split into 5.0 lbs. per hour of approximately 7 $\frac{3}{4}$  inch diameter ingot and 11.7 lbs. per hour of overflow product. The ingot lowering rate was 1.0 inch per hour, the stirrer rate was 43 r.p.m., and the distance between the liquid-solid interface and the bottom of the

## 8

stirrer was 10 inches. The following analyses were obtained:

| Element | Feed, p.p.m. | Prod p.p.m. | Overflow, p.p.m. |
|---------|--------------|-------------|------------------|
| Si..... | 540          | 200         | 700              |
| Fe..... | 600          | 200         | 800              |

The five foregoing specific examples have been selected to illustrate a fairly wide range in the several operating parameters with respect to impurities in the feed metal, production rate and purity of the product ingot. It will be appreciated that there is a relationship between purity of feed and purity of product so that with higher purity of the feed metal there will be higher purity in the product ingot. Again, with a given purity of feed metal, purity of the product will be influenced to some degree by production rate.

Example 1 illustrates operations in which we utilize the highest commercial grade of aluminum pig for the feed metal, using a low production rate and achieving a comparatively high product purity. Example 2 is illustrative of the application of my invention to casting of purified ingot from feed metal below presently acceptable commercial grade. Example 3 is illustrative of the application of my invention in a case where average grade pot metal is utilized. Example 4 illustrates conditions in which the feed purity is the same as in Example 1 but production rate has been multiplied many times. Example 5 is similar to Example 1.

The terms and expressions which I have employed are used in a descriptive and not a limiting sense, and I have no intention of excluding such equivalents of the invention described as fall within the scope of the claims.

I claim:

1. Method of continuous casting of aluminum ingot having throughout its length a purity continuously maintained at a substantially uniform level above the purity level of the molten feed metal which comprises feeding

40 molten metal into the inlet of a pass-through molding chamber, maintaining the molten condition of the metal in that part of the molding chamber which is nearest the inlet and maintaining a frozen condition of the metal in that part of the molding chamber which is nearest the outlet, continuously withdrawing the frozen portion from the outlet of the molding chamber while causing the molten portion to flow rapidly over the interface between the molten and frozen metal and withdrawing from the molding chamber at the molten metal side of the interface as casting progresses a substantial portion of the molten metal including metal which has flowed over the interface and contains a higher percentage of impurities than is present in the feed metal, the relationship between (a) rate of feeding molten metal, (b) rate of withdrawing the frozen portion from the molding chamber and (c) rate of withdrawing molten metal from the molding chamber, being maintained substantially constant each relative to the others.

60 2. Method of continuous casting of aluminum ingot having throughout its length a purity continuously maintained at a substantially uniform level above the purity level of the molten feed metal which comprises feeding molten metal into the inlet of a pass-through molding chamber, maintaining the molten condition of the metal in that part of the molding chamber which is nearest the inlet and maintaining a frozen condition of the metal in that part of the molding chamber which is nearest the outlet, and continuously withdrawing the frozen portion from the outlet of the molding chamber while stirring

70 the molten metal adjacent the interface between the molten and frozen metal and withdrawing from the molding chamber at the molten metal side of the interface as casting progresses a substantial portion of the molten metal including metal which has been stirred adjacent the

interface and contains a higher percentage of impurities than is present in the feed metal, the relationship between (a) rate of feeding molten metal, (b) rate of withdrawing the frozen portion from the molding chamber and (c) rate of withdrawing molten metal from the molding chamber, being maintained substantially constant each relative to the others.

3. Method according to claim 2 in which the stirring is performed in a manner that causes the molten metal adjacent the interface to rotate around the axis of the ingot while being drawn downwardly against the peripheral portions of the interface, thence inwardly toward said axis and upwardly away from central portions of the interface.

4. Method of continuous casting of aluminum ingot having throughout its length a purity continuously maintained at a substantially uniform level above the purity level of the molten feed metal which comprises feeding molten metal into the inlet of a pass-through molding chamber, maintaining the molten condition of the metal in that part of the molding chamber which is nearest the inlet and maintaining a frozen condition of the metal in that part of the molding chamber which is nearest the outlet, continuously withdrawing the frozen portion from the outlet of the molding chamber while causing the molten portion of the feed metal to flow rapidly over the interface between the molten and frozen metal and withdrawing a substantial portion of the molten metal from the molding chamber at the molten metal side of the interface as casting progresses, the relationship between (a) rate of feeding molten metal, (b) rate of withdrawing the frozen portion from the molding chamber and (c) rate of withdrawing molten metal from the molding chamber, being maintained substantially constant each relative to the others whereby a substantially uniform composition of the molten metal just above the interface is maintained with a resultant uniformity in purity of the ingot produced.

5. Apparatus for continuous casting of high purity metal ingot having throughout its length a purity continuously maintained at a substantially uniform level above the purity level of the molten feed metal which comprises a pass-through molding chamber having an inlet and an outlet spaced longitudinally thereof, means for

5

feeding molten metal into the inlet of said chamber, means for causing a portion of the feed metal to freeze at a point between said inlet and outlet, means for continuously withdrawing the frozen portion from the outlet of the molding chamber, stirring means for causing the molten portion of the feed metal to flow rapidly over the interface between the molten and frozen metal, and means for withdrawing from the molding chamber at the molten metal side of the interface as casting progresses a substantial portion of the molten metal including metal which has flowed over the interface and contains a higher percentage of impurities than is present in the feed metal.

10

6. Apparatus for continuous casting of high purity metal ingot having throughout its length a purity continuously maintained at a substantially uniform level above the purity level of the molten feed metal which comprises a pass-through molding chamber having an inlet and an outlet spaced longitudinally thereof, means for feeding molten metal into the inlet of said chamber, means for causing a portion of the feed metal to freeze at a point between said inlet and outlet, means for continuously withdrawing the frozen portion from the outlet of the molding chamber, means for stirring the molten feed metal adjacent the interface between the molten and frozen metal, and means for withdrawing from the molding chamber at the molten metal side of the interface as casting progresses a substantial portion of the molten metal including metal which has been stirred adjacent the interface and contains a higher percentage of impurities than is present in the feed metal.

20

7. Apparatus according to claim 6 in which the stirring means is constructed and arranged to rotate the feed metal adjacent the interface around the axis of the ingot while drawing the feed metal downwardly against the peripheral portions of the interface, thence inwardly toward said axis and upwardly away from central portions of the interface.

25

30

35

#### References Cited in the file of this patent

#### UNITED STATES PATENTS

|           |         |                |
|-----------|---------|----------------|
| 1,160,169 | Hering  | Nov. 16, 1915  |
| 2,013,653 | Hoke    | Sept. 10, 1935 |
| 2,708,297 | Zeigler | May 17, 1955   |
| 2,753,254 | Rick    | July 3, 1956   |